

Dec. 6, 1927.

1,651,535

T. S. McDERMOTT

METHOD OF MAKING A PILE FABRIC

Filed Dec. 27. 1926

Fig. 1.



Fig. 2.



Fig. 3.



Fig. 4.



Inventor.

Thomas S. McDermott

by Heard Smith & Tennant.

Atlys.

Patented Dec. 6, 1927.

1,651,535

# UNITED STATES PATENT OFFICE.

THOMAS S. McDERMOTT, OF FRANKLIN, MASSACHUSETTS, ASSIGNOR TO CLARK-CUTLER-McDERMOTT CO., OF FRANKLIN, MASSACHUSETTS, A CORPORATION OF MASSACHUSETTS.

## METHOD OF MAKING A PILE FABRIC.

Application filed December 27, 1926. Serial No. 157,081.

This invention relates to a method of making a pile fabric.

One of the objects of the invention is to provide a pile fabric which is inexpensive to manufacture but which is satisfactory for use as a rug and in various other ways in which pile fabrics are commonly used.

In accordance with the invention the pile fabric is formed by first attaching a layer 10 or ply of felt or unspun fibre to a fabric ply (such for instance as burlap) by pricking through both plies, this operation carrying some of the fibres of the unspun ply through and interlocking them with the fabric ply 15 and thus making a compound layer, and then applying to the fabric ply face of the compound layer another layer or ply of unspun fibres and subsequently pricking again through the compound layer and the second- 20 named ply of unspun fibres thereby to carry fibres from the first-named ply of unspun fibres through the fabric ply and into the second ply of unspun fibres. This second 25 ply of unspun fibres is subsequently stripped off from the fabric and in doing so the pile of the fabric is drawn up from the fabric face. The complete fabric thus when ready for use will have a bottom layer or ply of unspun fibres, a superposed fabric ply and 30 formed from fibres which have been drawn through the fabric ply.

In order to give an understanding of the invention I have illustrated in the drawings a selected embodiment thereof which will 35 now be described after which the novel features will be pointed out in the appended claims.

Figs. 1, 2 and 3 illustrate successive steps in the process of making the pile fabric;

40 Fig. 4 is a sectional view illustrating the pile fabric when completed.

The pile fabric shown in Fig. 4 comprises a bottom layer or ply 2 of unspun fibres, such for instance as felt, an upper ply 1 45 which is desirably in the nature of a coarse fabric, and a pile 3 which is formed by fibres of the unspun ply 2 which have been drawn through the fabric ply 1.

In making this type of fabric I first superpose a ply or layer 2 of unspun fibres, such for instance as felt, upon a fabric 1 and then subject the superposed layers or plies to the action of needles 5 which prick through the two plies and in doing so carry a portion of

the fibres of the unspun material 2 through 55 the fabric ply 1 as shown at 6, the fibres 6 projecting below the lower face of the fabric 1. This operation serves to unite the two plies 1 and 2 thus making a compound layer or fabric 10.

Another similar compound layer or fabric 11 is made as shown in Fig. 2 by laying a sheet 7 of unspun or felted fibres on a fabric ply 8 and then subjecting the superposed plies to the pricking operation of needles 5 65 as above described, which will cause some of the fibres of the ply 7 to be carried through and interlocked with the fabric 8 as shown at 9.

When the two compound layers or fabrics 70 have thus been formed they are superposed one on the other as shown at the left in Fig. 3, with the fabric-ply side of the compound layer 10 resting against the top face of the unspun ply 7 of the compound layer 11. 75 These superposed compound layers are then subjected to another pricking operation by means of the needles 5 and this pricking operation will carry additional fibres of the 80 ply 2 through the fabric 1 and will also carry said fibres into the fibrous ply 7 so that a large number of the fibres of the felt ply 2 which have been carried through the fabric 1 are interlocked with the felt ply 7.

After the fabric has been subjected to this 85 needling or pricking operation then the two compound fabrics or layers are pulled apart as shown at the right in Fig. 3. Inasmuch as the fibres which project through the fabric 1 are anchored well in the fibrous ply 7 this 90 operation of pulling the two compound fabrics apart will pull up a thick and long pile 3 on the face of the fabric 1. When the two compound fabrics are thus separated the pile fibres 3 which are pulled up from the 95 face of the fabric 1 are of different lengths thus making an irregular pile.

The fabric is finished by shearing the pile 3 so as to make an even pile as shown in Fig. 4.

100

I claim:

1. The method of making a pile fabric which consists in forming two compound layers each composed of a ply of unspun fibres anchored to a fabric ply, superposing 105 said compound layers with the fabric ply of one layer lying against the unspun ply of the other layer, pricking through both com-

- compound layers to carry fibres of one unspun  
5 ply through the intermediate fabric ply and  
into the other ply of unspun fibres and then  
pulling the two compound layers apart  
thereby pulling up a pile from the face of  
the fabric ply.
2. The method of making a pile fabric  
which consists in superposing two layers or  
plies of unspun fibre and a fabric ply with  
10 the fabric ply between those of the unspun  
fibres, pricking through the superposed plies  
to carry fibres from one ply of unspun  
fibres through the fabric ply and into the  
other ply of unspun fibres and then pulling  
the last-named ply from the fabric ply there-  
15 by to pull up a pile from the fibres after  
they have been pricked through the fabric  
ply.

In testimony whereof, I have signed my  
name to this specification.

THOMAS S. McDERMOTT.